# EUROPEAN PATENT SPECIFICATION

(11) **EP 2 403 982 B1**
(45) Date of publication and mention of the grant of the patent: **29.10.2014**
(21) Application number: 10749090.6
(22) Date of filing: 10.02.2010
(51) Int. Cl.: D02J 3/00, D01F 6/58, D01F 6/12

(54) **HYDROPHILIC FLUOROPOLYMER MATERIAL AND METHOD OF MAKING SAME**
HYDROPHILES FLUORPOLYMERMATERIAL UND HERSTELLUNGSVERFAHREN DAFÜR
MATIÈRE POLYMÈRE FLUORÉE HYDROPHILE ET SON PROCÉDÉ DE FABRICATION

(30) Priority: 03.03.2009 US 396749; 03.03.2009 US 396808; 03.03.2009 US 396776
(43) Date of publication of application: 11.01.2012
(73) Proprietor: Toray Fluorofibers (America) Inc., Decatur, AL 35601 (US)
(72) Inventor: DONCKERS, J., Michael, Decatur AL 35601 (US); NELSON, Artgur Russell, Decatur AL 35603 (US); MOON, Chester Darryl, Tuscumbia, AL 35674 (US)
(74) Representative: Dempster, Benjamin John Naftel
(86) International application number: PCT/US2010/023772
(87) International publication number: WO 2010/101701

(56) References cited:
- WO-A1-2005/017240
- JP-A- 7 070 920
- US-A- 5 700 572
- US-A1- 2006 051 574
- US-A1- 2007 190 880
- US-A1- 2007 275 618

## Description

### Technical Field

The present invention relates to a hydrophilic fluoropolymer material. More particularly, the invention relates to a fluoropolymer fiber floc or staple having a modified surface morphology giving rise to increased hydrophilicity.

### Background Art

Fluoropolymers have properties such as extremely low coefficient of friction, wear and chemical resistance, dielectric strength, temperature resistance and various combinations of these properties that make fluoropolymers useful in numerous and diverse industries. For example, in the chemical process industry, fluoropolymers are used for lining vessels and piping. The biomedical industry has found fluoropolymers to be biocompatible and so have used them in the human body in the form of both implantable parts and devices with which to perform diagnostic and therapeutic procedures. In other applications, fluoropolymers have replaced asbestos and other high temperature materials. Wire jacketing is one such example. Automotive and aircraft bearings, seals, push-pull cables, belts and fuel lines, among other components, are now commonly made with a virgin or filled fluoropolymer component.

In order to take advantage of the properties of fluoropolymers, fluoropolymers often must be modified by decreasing their lubricity in order to be bonded to another material. That is because the chemical composition and resulting surface chemistry of fluoropolymers render them hydrophobic and therefore notoriously difficult to wet. Hydrophobic materials have little or no tendency to adsorb water and water tends to "bead" on their surfaces in discrete droplets. Hydrophobic materials possess low surface tension values and lack active groups in their surface chemistry for formation of "hydrogen-bonds" with water. In the natural state, fluoropolymers exhibit these hydrophobic characteristics, which requires surface modification to render it hydrophilic. The applications mentioned above all require the fluoropolymer to be modified.

One such modification includes chemically etching the fluoropolymers. For example, fluoropolymer films and sheets are often etched on one side to enable bonding it to the inside of steel tanks and piping; the outside diameter of small diameter, thin wall fluoropolymer tubing is etched to bond to an over-extrusion resulting in a fluoropolymer-lined guide catheter for medical use; fluoropolymer jacketed high-temperature wire is etched to allow the printing of a color stripe or other legend such as the gauge of the wire and/or the name of the manufacturer; fluoropolymer based printed circuit boards require etching to permit the metallization of throughholes creating conductive vertical paths between both sides of a double sided circuit board or connecting several circuits in a multilayer configuration.

The first commercially viable processes were chemical in nature and involved the reaction between sodium and the fluorine of the polymer. In time, some of the chemistry was changed to make the process less potentially explosive and hazardous, but the essential ingredient - sodium - remains the most reliable, readily available chemical 'abrasive' for members of the fluoropolymer family.

In addition to being hazardous, chemically etched fluoropolymer surfaces tend to lose bond strength over time. It has been shown that temperature, humidity and UV light have a detrimental effect on etched surfaces. Tests have shown that etched fluoropolymer parts exposed to 250°F for 14 days exhibit bond strengths approximately 40% weaker than those done on the day they were etched. Further, depending upon the wavelength and intensity of the UV light source, the bond strength deterioration can occur over a period of months and years. It is thought that, due to the somewhat amorphous nature of these polymers, a rotational migration occurs over time, accelerated by some ambient conditions - especially heat ~ that re-exposes more of the original C2F4 molecule at the surface resulting in a lower coefficient of friction.

Another factor that is of concern with chemical etching of fluoropolymers is that of the depth of the etched layer. The sodium reaction with fluorine is a self-limiting one, and it has been shown to take place to a depth of only a few hundred to a few thousand Angstroms.

US2006/0051574 describes an existing fiber having increased filament separation and a method for making such a fiber.

### Disclosure of the Invention

The present invention is directed to a fluoropolymer fiber according to claim 1.

The tears may be formed by mechanically processing the material. One process may include placing a fluoropolymer material into an air stream and introducing mechanical energy into the material by colliding the material against itself. Another process may include cooling the fluoropolymer material, making the material brittle and then mechanically grinding it. It is believed that in most instances the tears are formed between the individual fluoropolymer particles that make up the material.

The surface modifications brought about by these processes may increase the surface area and roughness of the fluoropolymer materials. As a result, the lubricity of the material is decreased and the hydrophilicity is increased. This allows the fluoropolymer material to form long-lasting, homogenous slurries in aqueous solutions. It is believed that these modifications will allow the materials to be more easily mixed with resins and thermoplastics and molded into parts.

Other features of the present invention will become apparent from a reading of the following description, as well as a study of the appended drawings.

### Brief Description of the Drawings

FIG. 1 is a scanning electron micrograph ("SEM") of a virgin PTFE floc material, as prepared in Example 1.
FIG. 2 is a SEM of virgin PTFE floc material, as prepared in Example 1.
FIG. 3 is a SEM of a virgin PTFE floc material, as prepared in Example 1.
FIG. 4 is a SEM of a virgin PTFE floc material, as prepared in Example 1.
FIG. 5 is a SEM of a virgin PTFE floc material, as prepared in Example 2.
FIG. 6 is a SEM of a PTFE floe material according to the presently preferred embodiment of the present invention, as prepared in Example 3.
FIG. 7 is a SEM of a PTFE floc material according to the presently preferred embodiment of the present invention, as prepared in Example 3.
FIG. 8 is a SEM of a PTFE floc material according to the presently preferred embodiment of the present invention, as prepared in Example 3.
FIG. 9 is a SEM of a PTFE floc material according to the presently preferred embodiment of the present invention, as prepared in Example 3.
FIG. 10 is a SEM of a PTFE floc material according to the presently preferred embodiment of the present invention, as prepared in Example 3.
FIG. 11 is a SEM of a PTFE floc material according to the presently preferred embodiment of the present invention, as prepared in Example 3.
FIG. 12 is a SEM of a PTFE floc material according to the presently preferred embodiment of the present invention, as prepared in Example 3.
FIG. 13 is a SEM of a PTFE floc material according to the presently preferred embodiment of the present invention, as prepared in Example 3.
FIG. 14 is a SEM of a PTFE floc material according to the presently preferred embodiment of the present invention, as prepared in Example 3.
FIG. 15 is a SEM of a PTFE floc material according to the presently preferred embodiment of the present invention, as prepared in Example 4.
FIG. 16 is a SEM of a PTFE floc material according to the presently preferred embodiment of the present invention, as prepared in Example 4.
FIG. 17 is a SEM of a PTFE floc material according to the presently preferred embodiment of the present invention, as prepared in Example 4.
FIG. 18 is a SEM of a PTFE floc material according to the presently preferred embodiment of the present invention, as prepared in Example 4.
FIG. 19 is a SEM of a PTFE floc material according to the presently preferred embodiment of the present invention, as prepared in Example 4.
FIG. 20 is a SEM of a PTFE floc material according to the presently preferred embodiment of the present invention, as prepared in Example 4.

### Best Mode for Carrying Out Invention

The fluoropolymer material of the present invention is preferably prepared from a fluoropolymer fiber, such as continuous fluoropolymer filament yarn, which is made into floc or staple and processed in jet mill or a cryogenic grinder. In each process, the physical appearance of the fluoropolymer fibers is modified in a manner that improves the hydrophilicity of the material. This occurs by forming deformations in the fluoropolymer fibers that are visible using scanning electron microscopy at magnifications as low as X120. The deformations act to increase and roughen the surface area of the fibers by tearing the typically smooth exterior body and ends of the individual floc fibers and providing the fibers with split ends, slits along the bodies of the fibers, outwardly extending, fibril-like members, and exposed interior fiber portions.

In the present invention, by "fluoropolymer fiber" it is meant a fiber prepared from polymers such as polytetrafluoroethylene ("PTFE"), and polymers generally known as fluorinated olefinic polymers, for example, copolymers of tetrafluoroethylene and hexafluoropropene, copolymers of tetrafluoroethylene and perfluoroalkyl-vinyl esters such as perfluoropropyl-vinyl ether and perfluoroethyl-vinyl ether, fluorinated olefinic terpolymers including those of the above-listed monomers and other tetrafluoroethylene based copolymers. For the purposes of this invention, the preferred fluoropolymer fiber is PTFE fiber.

In the present invention, by "split" it is meant a tear that extends along a length of a fluoropolymer material and out through an end of the fiber. A spilt can appear as a crack through an end of the fiber or result in the formation of separated or partially separated fiber strands, each strand having a free end and an attached end. In some instances, the end of a fiber may include a single split thereby giving rise to a pair of strands, which may or may not have the same thickness. Alternatively, the end of a fiber may include many splits thereby giving rise to many strands. In this instance, the end of the fiber can have a frayed appearance depending on the number and lengths of the splits. A split typically does not result in the removal of material or a substantial amount of material from the fiber. However, in some instances, a split can extend along a length of a fiber and result in the complete removal of a sliver-like portion of the fiber, or along the entire length of the fiber thus removing a side of the fiber.

In the present invention, by "slit" it is meant a tear that extends partially along a length of a fluoropolymer fiber but does not extend through one of the opposing ends of the fiber. Slits often appear as an elongated, continuous openings that extend into an interior of the fiber to a particular depth. Like a split, a slit typically does not result in the removal of material or a substantial amount of material from the fiber.

In the present invention, by "grain" it is meant a longitudinal arrangement or pattern of fibril-like members. Often, a tear in the fluoropolymer fiber will expose an interior surface of the fiber. These interior surfaces can exhibit a grain running longitudinally along the axis of the fiber. The grain gives the exposed interior surface of the fiber the appearance of ridges extending lengthwise along the exposed interior surface.

In the present invention, by "fibril-like members" it is meant the elongated pieces that make up the grain of a fluoropolymer fiber. Under the various magnifications exhibited in the figures, the fibril-like members are not visible along a length of the exterior surface of the fibers. However, they are visible on the interior surfaces of the fluoropolymer fibers when the interior surfaces are exposed, for example, by a tear. When the fluoropolymer fiber is torn, exposing the interior surfaces of the fibers, a portion of the fibril-like members appear to become partially dislodged from the fibers and extend outwardly therefrom. These fibril-like members have attached ends and free ends which extend outwardly from exposed interior surfaces of the fluoropolymer fiber.

The fluoropolymer fiber of the present invention can be spun by a variety of means, depending on the exact fluoropolymer composition desired. Thus, the fibers can be spun by dispersion spinning; that is, a dispersion of insoluble fluoropolymer particles is mixed with a solution of a soluble matrix polymer and this mixture is then coagulated into filaments by extruding the mixture into a coagulation solution in which the matrix polymer becomes insoluble. The insoluble matrix material may later be sintered and removed by oxidative processes if desired. One method which is commonly used to spin PTFE and related polymers includes spinning the polymer from a mixture of an aqueous dispersion of the polymer particles and viscose, where cellulose xanthate is the soluble form of the matrix polymer, as taught for example in U.S. Pat. Nos. 3,655,853; 3,114,672 and 2,772,444. However, the use of viscose suffers from some serious disadvantages. For example, when the fluoropolymer particle and viscose mixture is extruded into a coagulation solution for making the matrix polymer insoluble, the acidic coagulation solution converts the xanthate into unstable xantheic acid groups, which spontaneously lose CS₂, an extremely toxic and volatile compound. Preferably, the fluoropolymer fiber of the present invention is prepared using a more environmentally friendly method than those methods utilizing viscose. One such method is described in U.S. Pat. Nos. 5,820,984; 5,762,846, and 5,723,081, which patents are incorporated herein in their entireties by reference. In general, this method employs a cellulosic ether polymer such as methylcellulose, hydroxyethylcellulose, methylhydroxypropylcellulose, hydroxypropylmethylcellulose, hydroxypropylcellulose, ethylcellulose or carboxymethylcellulose as the soluble matrix polymer, in place of viscose. Alternatively, if melt viscosities are amenable, filament may also be spun directly from a melt. Fibers may also be produced by mixing fine powdered fluoropolymer with an extrusion aid, forming this mixture into a billet and extruding the mixture through a die to produce fibers which may have either expanded or un-expanded structures. For the purposes of this invention, the preferred method of making the fluoropolymer fiber is by dispersion spinning where the matrix polymer is a cellulosic ether polymer.

The fluoropolymer fiber can be made into floc or staple using any number of means known in the art. Preferably, the fluoropolymer fiber is cut into floc or staple by a guillotine cutter, which is characterized by a to-and-fro movement of a cutting blade. Following cutting, the fluoropolymer fibers preferably have lengths ranging between 127 microns and 115,000 microns.

The process for modifying the physical appearance of the fluoropolymer materials by forming deformations in the fibers is achieved by introducing mechanical energy into the fluoropolymer fibers to such a degree that the ends of the fibers are split, slits are formed in the bodies of the fibers, a grain of the fiber is exposed, and fibril-like members are extended outwardly from exposed interior surface portions of the fibers. Preferably, the processes do not substantially decrease the length of the individual fibers.

One suitable process includes entraining the fibers in an air stream, directing the entrained fibers through an orifice and colliding the pieces into one another. This process is preferably carried out using a jet mill and jet milling processes, examples of which are described in U.S. Pat. Nos. 7,258,290; 6,196,482, 4,526,324; and 4,198,004. Another suitable process includes cooling the fluoropolymer fibers to a cryogenic temperature of about -268°C or less, depending on the low temperature embrittlement properties of the particular fibers, and then grinding the fibers. This process is preferably carried out using a cryogrinder and cryogrinding processes, examples of which are described in U.S. Pat. Nos. 4,273,294; 3,771,729; and 2,919,862.

Jet mills and cryogrinders are conventionally used to pulverize materials into fine particles or powder. For example, jet milling is a process that uses high pressure air to micronize friable, heat-sensitive materials into ultra-fine powders. Powder sizes vary depending on the material and application, but typically ranges from 75 to as fine as 1 micron can be prepared. Often materials are jet milled when they need to be finer than 45 microns. Cryogenic grinding is a process that uses liquid nitrogen to freeze the materials being size-reduced and one of a variety of grinding mechanisms to ground them to a powder distribution depending on the application. Particle sizes of 0.1 micron can be obtained. However, it has unexpectedly been found that jet or cryogenic milling can be carried out on the fluoropolymers materials of the present invention without the materials being pulverized or size-reduced. More particularly, it has been found that the materials can be processed with a jet mill or a cryogenic grinding mill without substantially affecting the lengths of fibers, while at the same time forming splits in the ends of the fibers, forming slits in the bodies of the fibers, forming outwardly extending, fibril-like members and exposing the interior surfaces of the materials. Also, unexpectedly, these modifications have been found to render the processed fluoropolymer materials hydrophilic thus converting a hydrophobic material into a hydrophilic material, or in the alternative, increasing or improving the hydrophilicity of the materials.

The present invention will be explained further in detail by the following Examples. In each of the Examples, a 6.7 denier per filament continuous, cellulosic ether-based PTFE filament yarn was prepared and cut with a guillotine cutter into virgin floc.

### EXAMPLE 1

In Example 1, the virgin floc was cut into lengths of approximately 200 to 250 microns. As displayed in FIGS. 1 through 4, the virgin floc fibers had smooth, nearly featureless exterior surfaces along the lengths thereof. The ends of the floc fibers were substantially smooth and nearly featureless as well, with the exception of the PTFE floc fibers shown in FIG. 4, which exhibited some uneven areas which are believed to have resulted from the cutting process.

The wettability of the 200 to 250 microns virgin PTFE fiber floc was tested. In a first test, 50 grams of the floc and 200 ml of deionized water were placed into a Waring blender and mixed for 30 seconds. Thereafter, the mixture was observed. Immediately, the PTFE floc fibers that were not adhered to the walls of the blender or floating on top of the water began to settle to the bottom of the blender. This resulted in the formation of three distinct mixture portions including a floc rich bottom portion, a water rich middle portion and a top portion composed of PTFE fiber floc floating on top of the middle portion. The floc in the top portion appeared dry.

In a second test, the wettability of the PTFE fiber floc was determined by placing 50 grams of the floc and 200 ml of deionized water into a Waring blender, mixing the water and fibers for 30 seconds and immediately thereafter siphoning a portion of the mixture into a syringe. As in the first test, the PTFE floc fibers quickly settled into three portions including a floc rich bottom portion, a water rich middle portion and a top portion composed of floc fibers floating on top of the middle portion.

The results evidenced that the 200 to 250 microns virgin PTFE fiber floc was hydrophobic.

### EXAMPLE 2

In Example 2, the virgin floc was cut into lengths of approximately 6350 microns. As displayed in FIG. 5, the virgin floc fibers had smooth, nearly featureless exterior surfaces along the lengths thereof. These figures further show that floc fibers tended to clump together.

The wettability of the 6350 microns virgin PTFE fiber floc was tested. Fifty grams of the floc and 200 ml of deionized water were placed into a Waring blender and mixed for 30 seconds. Thereafter, the mixture was observed. Immediately, the PTFE floc fibers began to settle to the bottom of the container. This resulted in the formation of two distinct mixture portions including a floc rich bottom portion and a water rich top portion

The test results evidenced that the 6350 microns PTFE fiber floc was hydrophobic.

### EXAMPLE 3

In Example 3, a portion of the 200 to 250 microns virgin PTFE fiber floc was processed by jet milling and examined. As shown in FIGS. 6 through 14, jet mill processing of the fluoropolymer fiber floc modified the physical appearance of the fluoropolymer fibers. The modifications included surface deformations caused by tearing of the fibers. The tearing resulted in the formation of split fiber ends, slits along the bodies of the fibers, and formation of outwardly extending, fibril-like members and the exposure of interior surfaces of the fibers. The exposed interior surfaces of the fibers exhibited a grain that in certain instances, where a split resulted in the removal of an entire side of the fiber, extended the entire length of the fibers. The grain appeared to be formed by the fibril-like members.

The majority of the fibril-like members remained fully coupled to the fiber surfaces after tearing thus providing the exposed interior surfaces with a number of longitudinally extending ridges. The ridges gave the exposed interior surfaces a rough appearance in contrast to the smooth exterior surfaces of the fibers. In other instances, the fibril-like members became partially detached from the fibers and extended outwardly from the fiber surfaces. These fiber surfaces primarily included the exposed interior surfaces but also included areas along the edges formed between the exterior surfaces and exposed interior surfaces of the fibers. An example of an exposed interior surface is well depicted in FIGS. 6, 7 and 12. It is believed that the fibril-like members constitute individual or small groupings of elongated or drawn PTFE particles. The partially detached fibril-like members were often bent or curved and had lengths in excess of 100 microns.

The slits appeared to form between groupings of the fibril-like members and individual fibril-like members. The observed members had lengths that were less than 20 microns and as long as 80 microns. The depth of the of the slits was difficult to determine, but it was found that some of the slits extended through the entire thickness or width of the PTFE fibers. A plurality of slits formed within a single fiber are well depicted in FIG. 8.

FIGS. 10 through 13 depict various splits through the ends of the PTFE fibers. A typical frayed fiber end is shown in FIG. 10, the fiber being frayed at both ends. The frayed portions are exhibited as individual strands having free ends and ends attached to the fiber. The fiber in FIG. 10 also appears to have had an entire side of the fiber split off from the fiber thus exposing an interior surface of the fiber that extends the length of the fiber. This occurrence is also depicted in FIGS. 6 and 7. FIG. 11 provides an example of a split that does not result in a strand having a free end but rather appears as a crack that extends through the end of the fiber.

The splits ranged in lengths from less than 1 micron to the entire length of the fibers. In those instances where substantial fraying was observed, the fiber ends included splits in the range of 50 to 75 microns.

The wettability of the jet milled, 200 to 250 microns PTFE fiber floc was tested. In a first test, 50 grams of the processed floc and 200 ml of deionized water were placed into a Waring blender and mixed for 30 seconds. Thereafter, the mixture was observed. The mixture appeared as a homogenous, aqueous dispersion of the fluoropolymer floc. No floc was observed settling at the bottom of the container, and none of the floc was observed floating on top of the mixture. The mixture maintained a homogenous state for several days even as the amount of water in the container decreased by evaporation. Eventually, enough water evaporated from the container that the wetted fluoropolymer floc took on the consistency of dough.

In a second test, the wettability of the jet milled PTFE fiber floc was determined by placing 50 grams of the processed floc and 200 ml of deionized water into a Waring blender, mixing the water and fibers for 30 seconds and immediately thereafter siphoning a portion of the mixture into a syringe. As in the first test, the mixture appeared as a homogenous, aqueous dispersion of fluoropolymer floc. No floc was observed settling at the bottom of the syringe, and none of the floc was observed floating on top of the mixture. The homogenous slurry flowed easily into and out of syringe on multiple occasions exhibiting excellent flow characteristics

The tests results evidence that the jet milled, 200 to 250 microns PTFE fiber floc was hydrophilic.

### EXAMPLE 4

In Example 4, a portion of the 6350 microns virgin PTFE fiber floc was processed by cryogenic grinding and examined. As shown in FIGS. 15 through 20, cryogenic milling of the fluoropolymer fiber floc modified the physical appearance of the fluoropolymer fibers much like jet milling. Thus, the cryogenic milled fibers included split fiber ends, slits along the bodies of the fibers, formation of outwardly extending, fibril-like members and exposure of interior surfaces of the fibers. No substantial differences in the surface morphology of the fibers milled by the cryogenic grinding process and the jet milling processing were observed.

The wettability of the cryogenic milled, 6350 microns PTFE fiber floc was tested. Fifty grams of the processed floc and 200 ml of deionized water were placed into a Waring blender and mixed for 30 seconds. Thereafter, the mixture was observed. The mixture appeared as a homogenous, aqueous dispersion of the fluoropolymer floc. No floc was observed settling at the bottom of the container, and none of the floc was observed floating on top of the mixture. For reasons unknown, the cryogenic milled floc dispersed throughout the aqueous medium and provided the mixture with a sponge-like consistency.

The tests results evidence that the cryogenic milled, 6350 microns PTFE fiber floc was hydrophilic.

As will be apparent to one skilled in the art, various modifications can be made within the scope of the aforesaid description. Such modifications being within the ability of one skilled in the art form a part of the present invention and are embraced by the claims below.

## Claims

1. A fluoropolymer fiber comprising an improved hydrophilicity and a surface deformation configured for providing the improved hydrophilicity, wherein the surface deformation is a slit having a depth that is greater than 10% of an average width of the fluropolymer fiber,
wherein the slit is a tear that extends partially along a length of a fluoropolymer fiber but does not extend through one of the opposing ends of the fiber.

2. The fluoropolymer fiber according to claim 1, wherein the fiber also includes surface deformation which is a split or a plurality of splits which preferably form a plurality of strands which may provide an end of the fluoropolymer fiber with a frayed appearance.

3. The fluoropolymer fiber according to claim 2, wherein the split has a length that is equal to between 1% and 100% of a length of the fluoropolymer fiber, and the surface deformation may be a tear having a length that is equal to between 5% and 90% of a length of the fluoropolymer fiber and preferably the surface deformation is a tear having a length that is equal to between 10% and 80% of a length of the fluoropolymer fiber.

4. The fluoropolymer fiber according to claim 1, 2 or 3, wherein the surface deformation extends along a grain of the fluoropolymer fiber and/or the surface deformation extends substantially longitudinally along an exterior surface of the fluoropolymer fiber.

5. The fluoropolymer fiber according to any preceding claim, wherein the surface deformation includes an exposed interior surface of the fluoropolymer fiber and optionally the exposed interior surface includes a fibril-like member extending outwardly therefrom and optionally the fibril-like member is bent.

6. The fluoropolymer fiber according to any preceding claim, wherein the improved hydrophilicity is UV light resistant and/or resistant to humidity and/or resistant to temperature.

7. The fluoropolymer fiber according to any preceding claim, wherein the fluoropolymer fiber is a polytetrafluoroethylene fiber between about 127 microns and about 1115,000 microns in length.

8. The fluoropolymer fiber according to any preceding claim, wherein the second surface deformation is a tear having a depth that is greater than 0.5 micron or greater than 2.5 microns.

9. The fluoropolymer fiber according to any preceding claim, wherein the second surface deformation is a slit having a depth that is greater than 10% of an average width of the fluoropolymer fiber or greater than 25% of an average width of the fluoropolymer fiber.

10. A fluoropolymer fiber according to any preceding claim, comprising,
an elongate body having a first end and a second end, and a
split extending through the first end of the elongate body.

11. The fluoropolymer fiber according to claim 10, wherein the split includes a first elongate portion partially removed from a surface of the elongate body, the first elongate portion having a first end coupled to the elongate body and a second free end and optionally the split includes a second portion including an exposed interior surface of the elongate body and optionally the exposed interior surface is rougher than an exterior surface of the fluoropolymer fiber and includes a plurality of outwardly extending, fibril-like, curved members.

12. The fluoropolymer fiber according to claim 10 or claim 11, wherein the split extends through the second end

13. The fluoropolymer fiber according to claim 10, 11 or 12, wherein the split has a length that is equal to between 2% and 75% of a length of the fluoropolymer fiber, and preferably the split has a length that is equal to between 15% and 60% of a length of the fluoropolymer fiber.

14. The fluoropolymer fiber according to any preceding claim, wherein the slit has a depth that is greater than 0.75 micron, preferably greater than 2.0 microns.

15. The fluoropolymer fiber according to any preceding claim, wherein the fluoropolymer fiber is a polytetrafluoroethylene fiber.

16. The fluoropolymer fiber according to any preceding claim wherein the fluropolymer fiber is a floc fiber or a staple fiber.

17. A hydrophilic fluoropolymer fiber as claimed in any of claims 10 to 16, the fiber including a split end, an exposed interior fluoropolymer fiber surface and a plurality of fibril-like members extending outwardly from the exposed interior surface.

18. The fluoropolymer fiber according to claim 17, wherein the slit has a depth of at least 0.8 micron.

19. The fluoropolymer according to claim 17 or claim 18, wherein the split has a length that is equal to between 10% and 100% of a length of the fluoropolymer fiber and/or the split end appears frayed.

20. The fluoropolymer fiber according to any of claims 17 to 19, wherein the fluoropolymer floc is an expanded fluoropolymer fiber or a polytetrafluoroethylene floc fiber or a polytetrafluoroethylene staple fiber.

21. A method for increasing the hydrophilicity of fluoropolymer fibers comprising mechanically modifying the fluoropolymer fibers to create surface deformation configured for providing the improved hydrophilicity, wherein the surface deformation is a slit having a depth that is greater than 10% of an average width of the fluoropolymer fiber,
wherein the slit is a tear that extends partially along a length of fluoropolymer fiber but does not extend through one of the opposing ends of the fiber.

22. The method according to claim 21, wherein the mechanically modifying is carried out by colliding the fluoropolymer fibers together and optionally the mechanically modifying is carried out by entraining the fluoropolymer fibers within a jet of air and optionally the mechanically modifying is carried out by a jet mill.

23. The method according to claim 21 or claim 22, wherein the mechanically modifying includes tearing the fluoropolymer fibers and may include partially removing exterior surface portions of the fluoropolymer fibers and optionally the exterior surface portions remain coupled at one end thereof to the fluoropolymer fibers from which they are partially removed.

24. The method according to claim 21 or claim 22, wherein the mechanically modifying includes splitting the fluoropolymer fibers into strands and/or imparting a rough exposed surface on a portion of the fluoropolymer fibers.

25. The method according to any of claims 21 to 24, wherein the mechanically modifying is carried out by impacting the fluoropolymer fibers with a jet of air.

26. The method according to any of claims 21 to 25 wherein the fluoropolymer fibers are flock fiber, staple fibers or combinations thereof.

27. The method according to any of claims 21 to 26, wherein the mechanically modifying includes forming a split in an end of at least one of the fluoropolymer fibers, the split having a length that is equal to between 5% and 100% of a length of the at least one fluoropolymer fiber, or optionally the mechanically modifying includes forming a split in an end of at least one of the fluoropolymer fibers, the split having a length that is equal to between 10% and 90% of a length of the at least one fluoropolymer fiber or optionally the mechanically modifying includes forming split in an end of at least one of the fluoropolymer fibers, the split having a length that is equal to between about 20% and about 50% of a length of the at least one fluoropolymer fiber.

28. The method according to any of claims 21 to 27, wherein the mechanically modifying includes forming a tear in at least one of the fluoropolymer fibers, the tear having a depth that is greater than 1.0 micron, preferably greater than 5.0 microns.

29. The method according to any of claims 21 to 28, wherein the mechanically modifying includes forming a plurality of fibril-like members that extend outwardly from an exposed interior surface of at least one of the fluoropolymer fibers and/or the mechanically modifying does not substantially shorten a total length of a majority of the fluoropolmer fibers.

30. The method according to any of claims 21 to 29, wherein the processing includes forming at least one tear within a surface of the fluoropolymer fiber, and the at least one tear extends substantially longitudinally along the surface of the fluoropolymer fiber and optionally forming the at least one tear includes exposing a plurality of underlying, substantially aligned, fluoropolymer particles.

31. The method according to any of claims 21 to 29, wherein the processing includes splitting an end of the fluoropolymer fiber into a plurality of strands and optionally the processing includes splitting an end of the fluoropolymer fiber along a grain thereof into a plurality of strands.

32. The method according to any of claims 21 to 31, wherein the processing includes converting a smooth surface portion of the fluoropolymer fiber to a rough surface portion and optionally the rough surface portion extends longitudinally along the fluoropolymer fiber.

33. A method as claimed in any of claims 21 to 32, comprising imparting hydrophilicity to the fluoropolymer material by mechanically milling the fluoropolymer material and optionally the mechanical milling includes directing a jet of air into the fluoropolymer material and optionally the mechanical milling includes driving the fluoropolymer material through an orifice of a jet mill with at least one jet of air.

34. The method according to claim 33, wherein the mechanical milling includes splitting at least one end of a portion of the fluoropolymer material into separate strands, and/or wherein the mechanical milling includes imparting a rough exposed surface to a portion of the fluoropolymer material and optionally the rough exposed surface extends along a longitudinal axis of the fluoropolymer material.

35. The method according to any of claims 21 to 34, wherein the fluoropolymer material includes polytetrafluoroethylene fibers.

## Patentansprüche

1. Fluorpolymer-Faser mit einer verbesserten hydrophilen Eigenschaft und einer Oberflächenverformung, welche ausgestaltet ist, die verbesserte hydrophile Eigenschaft bereit zu stellen, wobei die Oberflächenverformung ein Schlitz ist, welcher eine Tiefe aufweist, die größer als 10 % einer durchschnittlichen Breite der Fluorpolymer-Faser ist,
wobei der Schlitz ein Riss ist, welcher sich teilweise entlang einer Länge der Fluorpolymer-Faser erstreckt und welcher sich aber nicht durch eines der sich gegenüber liegenden Enden der Faser erstreckt.

2. Fluorpolymer-Faser nach Anspruch 1, wobei die Faser auch eine Oberflächenverformung aufweist, welche ein Schlitz oder eine Anzahl an Schlitzen ist, welche vorzugsweise eine Anzahl an Strängen bilden, welche an einem Ende der Fluorpolymer-Faser mit einem ausgefransten Erscheinungsbild vorgesehen sein können.

3. Fluorpolymer-Faser nach Anspruch 2, wobei der Schlitz eine Länge aufweist, welche gleich zwischen 1 % und 100 % einer Länge der Fluorpolymer-Faser ist, und wobei die Oberflächenverformung ein Riss sein kann, welcher eine Länge aufweist, die gleich wischen 5 % und 90 % einer Länge der Fluorpolymer-Faser ist, und wobei vorzugsweise die Oberflächenverformung ein Riss ist, welcher eine Länge aufweist, die gleich wischen 10 % und 80 % einer Länge der Fluorpolymer-Faser ist.

4. Fluorpolymer-Faser nach Anspruch 1, 2 oder 3, wobei die Oberflächenverformung sich entlang eines Kornes der Fluorpolymer-Faser erstreckt und / oder die Oberflächenverformung sich im Wesentlichen longitudinal entlang einer äußeren Oberfläche der Fluorpolymer-Faser erstreckt.

5. Fluorpolymer-Faser nach einem der vorhergehenden Ansprüche, wobei die Oberflächenverformung eine freiliegende innere Oberfläche der Fluorpolymer-Faser aufweist, und wobei vorzugsweise die freiliegende innere Oberfläche ein faserartiges Element aufweist, welches sich nach außen davon erstreckt, und wobei vorzugsweise das faserartige Element gebogen ist.

6. Fluorpolymer-Faser nach einem der vorhergehenden Ansprüche, wobei die verbesserte hydrophile Eigenschaft eine Beständigkeit gegenüber ultraviolettem Licht ist und / oder eine Beständigkeit gegenüber Feuchtigkeit ist und / oder eine Beständigkeit gegenüber Temperaturen ist.

7. Fluorpolymer-Faser nach einem der vorhergehenden Ansprüche, wobei die Fluorpolymer-Faser eine Polytetrafluoräthylen-Faser mit einer Länge wischen ungefähr 127 Mikrometern und ungefähr 1.115.000 Mikrometern ist.

8. Fluorpolymer-Faser nach einem der vorhergehenden Ansprüche, wobei die zweite Oberflächenverformung ein Schlitz ist, welcher eine Tiefe aufweist, die größer als 0,5 Mikrometer oder größer als 2,5 Mikrometer ist.

9. Fluorpolymer-Faser nach einem der vorhergehenden Ansprüche, wobei die zweite Oberflächenverformung ein Schlitz ist, welcher eine Tiefe aufweist, die größer als 10 % einer durchschnittlichen Breite der Fluorpolymerfaser ist oder die größer als 25 % einer durchschnittlichen Breite der Fluorpolymerfaser ist.

10. Fluorpolymer-Faser nach einem der vorhergehenden Ansprüche aufweisen: einen länglichen Körper, welcher ein erstes Ende und ein zweites Ende aufweist, und einem Schlitz, welcher sich durch das erste Ende des länglichen Körpers erstreckt.

11. Fluorpolymer-Faser nach Anspruch 10, wobei der Schlitz einen ersten länglichen Bereich aufweist, welcher teilweise von einer Oberfläche des länglichen Körpers entfernt ist, wobei der erste längliche Bereich ein erstes Ende, welches mit dem länglichen Körper verbunden ist, und ein zweites freies Ende aufweist, und wobei vorzugsweise der Schlitz einen zweien Bereich aufweist, welcher eine freiliegende innere Oberfläche des länglichen Körpers aufweist, und wobei vorzugsweise die freiliegende innere Oberfläche rauer als eine äußere Oberfläche der Fluorpolymer-Faser ist und eine Anzahl an sich nach außen erstreckenden, faserartigen, gekrümmten Elementen aufweist.

12. Fluorpolymer-Faser nach Anspruch 10 oder 11, wobei der Schlitz sich durch das zweite Ende erstreckt.

13. Fluorpolymer-Faser nach Anspruch 10, 11 oder 12, wobei der Schlitz eine Länge aufweist, welche gleich zwischen 2 % und 75 % einer Länge der Fluorpolymer-Faser ist, und wobei vorzugsweise der Schlitz eine Länge aufweist, welche gleich wischen 15 % und 60 % einer Länge der Fluorpolymer-Faser ist.

14. Fluorpolymer-Faser nach einem der vorhergehenden Ansprüche, wobei der Schlitz eine Tiefe aufweist, die größer als 0,75 Mikrometer ist und vorzugsweise größer als 2,0 Mikrometer ist.

15. Fluorpolymer-Faser nach einem der vorhergehenden Ansprüche, wobei die Fluorpolymer-Faser eine Polytetrafluorethylen-Faser ist.

16. Fluorpolymer-Faser nach einem der vorhergehenden Ansprüche, wobei die Fluorpolymer-Faser eine Flockenfaser oder eine Stapelfaser ist.

17. Hydrophile Fluorpolymer-Faser nach einem der Ansprüche 10 bis 16, wobei die Faser ein Ende des Schlitzes, eine freiliegende innere Oberfläche der Fluorpolymer-Faser und eine Anzahl an faserartigen Elementen aufweist, welche sich nach außen von der freiliegenden inneren Oberfläche erstrecken.

18. Fluorpolymer-Faser nach Anspruch 17, wobei der Schlitz eine Tiefe von mindestens 0,8 Mikrometern aufweist.

19. Fluorpolymer-Faser nach Anspruch 17 oder 18, wobei der Schlitz eine Länge aufweist, welche gleich zwischen 10 % und 100 % einer Länge der Fluorpolymer-Faser ist, und / oder das Ende des Schlitzes ausgefranzt ausgebildet ist.

20. Fluorpolymer-Faser nach einem der Ansprüche 17 bis 19, wobei die Fluorpolymer-Flocke eine expandierte Fluorpolymer-Faser oder eine Polytetrafluoräthylen-Flockenfaser oder eine Polytetrafluoräthylen-Stapelfaser ist.

21. Verfahren zur Verbesserung der hydrophilen Eigenschaft von Fluorpolymer-Fasern aufweisend: ein mechanisches Abändern der Fluorpolymer-Fasern, um eine Oberflächenverformung zu erzeugen, welche ausgestaltet ist, die verbesserte hydrophile Eigenschaft bereit zu stellen, wobei die Oberflächenverformung ein Schlitz ist, welcher eine Tiefe aufweist, die größer als 10 % einer durchschnittlichen Breite der Fluorpolymerfaser ist,
wobei der Schlitz ein Riss ist, welcher sich teilweise entlang einer Länge der Fluorpolymer-Faser erstreckt und welcher sich aber nicht durch eines der sich gegenüber liegenden Enden der Faser erstreckt.

22. Verfahren nach Anspruch 21, wobei das mechanische Abändern durchgeführt wird, indem die Fluorpolymer-Fasern zusammengestoßen, und wobei vorzugsweise das mechanische Abändern durchgeführt wird, indem die Fluorpolymer-Fasern in einem Luftstrom mitgeführt werden, und wobei vorzugsweise das mechanische Abändern mittels einer Strahlmühle durchgeführt wird.

23. Verfahren nach Anspruch 21 oder 22, wobei das mechanische Abändern ein Schlitzen der Fluorpolymer-Fasern aufweist und ein teilweise Entfernen von äußeren Oberflächenbereichen der Fluorpolymer-Fasern aufweisen kann und wobei vorzugsweise die äußeren Oberflächenbereiche der Fluorpolymer-Fasern mit einem von deren Ende mit den Fluorpolymer-Fasern verbunden bleiben, von denen sie teilweise entfernt worden sind.

24. Verfahren nach Anspruch 21 oder 22, wobei das mechanische Abändern ein Reißen der Fluorpolymer-Fasern in Stränge und / oder ein Aufbringen einer rauen Oberfläche auf einem Bereich der Fluorpolymer-Fasern aufweist.

25. Verfahren nach einem der Ansprüche 21 bis 24, wobei das mechanische Abändern durchgeführt wird, indem auf die Fluorpolymer-Fasern ein Luftstrom einwirkt.

26. Verfahren nach einem der Ansprüche 21 bis 25, wobei die Fluorpolymer-Fasern Flockenfasern oder Stapelfasern oder eine Kombination davon sind.

27. Verfahren nach einem der Ansprüche 21 bis 26, wobei das mechanische Abändern ein Bilden eines Schlitzes in einem Ende von wenigstens einer der Fluorpolymer-Fasern aufweist, wobei der Schlitz eine Länge aufweist, welche gleich zwischen 5 % und 100 % einer Länge der weinigstens einen Fluorpolymer-Faser ist, oder wobei vorzugsweise das mechanische Abändern ein Bilden eines Schlitzes in einem Ende von weinigstens einer der Fluorpolymer-Fasern aufweist, wobei der Schlitz eine Länge aufweist, welche gleich zwischen 10 % und 90 % einer Länge der weinigstens einen Fluorpolymer-Faser ist, oder wobei vorzugsweise das mechanische Abändern ein Bilden eines Schlitzes in einem Ende von weinigstens einer der Fluorpolymer-Fasern aufweist, wobei der Schlitz eine Länge aufweist, welche gleich zwischen 20 % und 50 % einer Länge der weinigstens einen Fluorpolymer-Faser ist.

28. Verfahren nach einem der Ansprüche 21 bis 27, wobei das mechanische Abändern ein Bilden eines Risses in weinigstens einer der Fluorpolymer-Fasern aufweist, wobei der Riss eine Tiefe aufweist, welche größer als 1,0 Mikrometer ist und vorzugsweise welche größer als 5,0 Mikrometer ist.

29. Verfahren nach einem der Ansprüche 21 bis 28, wobei das mechanische Abändern ein Bilden einer Anzahl von faserartigen Elementen aufweist, welche sich nach außen von einer freiliegenden inneren Oberfläche von weinigstens einer der Fluorpolymer-Fasern erstrecken, und / oder das mechanische Abändern eine Gesamtlänge von einer Mehrzahl der Fluorpolymer-Fasern im Wesentlichen nicht verkürzt.

30. Verfahren nach einem der Ansprüche 21 bis 29, wobei die Bearbeitung ein Bilden von weinigstens einem Riss innerhalb einer Oberfläche der Fluorpolymer-Fasern aufweist, und der weinigstens eine Riss sich im Wesentlichen longitudinal entlang der Oberfläche der Fluorpolymer-Faser erstreckt, und wobei vorzugsweise das Bilden von weinigstens einem Riss ein Freilegen einer Anzahl der zu Grunde liegenden, im Wesentlichen ausgerichteten Fluorpolymer-Partikel aufweist.

31. Verfahren nach einem der Ansprüche 21 bis 29, wobei die Bearbeitung ein Schlitzen eines Endes der Fluorpolymer-Faser in eine Anzahl an Strängen aufweist, und wobei vorzugsweise die Bearbeitung ein Schlitzen eines Endes der Fluorpolymer-Faser entlang eines Kornes davon in eine Anzahl an Strängen aufweist.

32. Verfahren nach einem der Ansprüche 21 bis 31, wobei die Bearbeitung ein Umwandern eines glatten Oberflächenbereiches der Fluorpolymer-Faser in einen rauen Oberflächenbereich aufweist und wobei vorzugsweise der raue Oberflächenbereich sich longitudinal entlang der Fluorpolymer-Faser erstreckt.

33. Verfahren nach einem der Ansprüche 21 bis 32 aufweisend: ein Aufbringen einer hydrophilen Eigenschaft auf das Fluorpolymer-Material, indem das Fluorpolymer-Material mechanisch gemahlen wird, und wobei vorzugsweise das mechanische Mahlen ein Führen eines Luftstromes auf das Fluorpolymer-Material aufweist, und wobei vorzugsweise das mechanische Mahlen ein Treiben des Fluorpolymer-Materials durch eine Öffnung einer Strahlmühle mit wenigstens einem Luftstrom aufweist.

34. Verfahren nach Anspruch 33, wobei das mechanische Mahlen ein Schlitzen von wenigstens einem Ende eines Bereiches des Fluorpolymer-Materials in einzelne Stränge aufweist, und / oder wobei das mechanische Mahlen ein Aufbringen einer rauen freiliegenden Oberfläche auf einen Bereich des Fluorpolymer-Materials aufweist, und wobei vorzugsweise die raue freiliegende Oberfläche sich entlang einer longitudinalen Achse des Fluorpolymer-Materials erstreckt.

35. Verfahren nach einem der Ansprüche 21 bis 34, wobei das Fluorpolymer-Material Polytetrafluoräthylen-Fasern aufweist.

## Revendications

1. Fibre polymère fluorée présentant une hydrophilicité améliorée et une déformation de surface configurée pour procurer l'hydrophilicité améliorée, **caractérisée en ce que** la déformation de surface est une fente ayant une profondeur qui est supérieure à 10% d'une largeur moyenne de la fibre polymère fluorée, et **en ce que** la fente est une déchirure qui s'étend partiellement le long d'une fibre polymère fluorée, mais qui ne s'étend pas à travers une des extrémités opposées de la fibre.

2. Fibre polymère fluorée selon la revendication 1, **caractérisée en ce que** la fibre présente également une déformation de surface qui est une fente ou une multiplicité de fentes qui forment de préférence une multiplicité de brins, qui peuvent donner à une extrémité de la fibre polymère fluorée un aspect effiloché.

3. Fibre polymère fluorée selon la revendication 2, **caractérisée en ce que** la fente présente une longueur qui est comprise entre 1% et 100% de la longueur de la fibre polymère fluorée, et la déformation de surface peut être une déchirure qui présente une profondeur qui est comprise entre 5% et 90% de la longueur de la fibre polymère fluorée et la déformation de surface est de préférence une déchirure présentant une longueur qui est comprise entre 10% et 80% de la longueur de la fibre polymère fluorée.

4. Fibre polymère fluorée selon la revendication 1, 2 ou 3, **caractérisée en ce que** la déformation de surface s'étend le long d'un grain de la fibre polymère fluorée et/ou la déformation de surface s'étend sensiblement en direction longitudinale le long d'une surface extérieure de la fibre polymère fluorée.

5. Fibre polymère fluorée selon l'une quelconque des revendications précédentes, **caractérisée en ce que** la déformation de surface comprend une surface intérieure exposée de la fibre polymère fluorée et en option la surface intérieure exposée comprend un élément de type fibrille s'étendant vers l'extérieur à partir de celle-ci et en option l'élément de type fibrille est courbé.

6. Fibre polymère fluorée selon l'une quelconque des revendications précédentes, **caractérisée en ce que** l'hydrophilicité améliorée est résistante à la lumière UV et/ou résistante à l'humidité et/ou résistante à la température.

7. Fibre polymère fluorée selon l'une quelconque des revendications précédentes, **caractérisée en ce que** la fibre polymère fluorée est une fibre de polytétrafluoroéthylène d'une longueur comprise entre environ 127 microns et environ 1115.000 microns.

8. Fibre polymère fluorée selon l'une quelconque des revendications précédentes, **caractérisée en ce que** la seconde déformation de surface est une déchirure présentant une profondeur qui est supérieure à 0,5 microns ou supérieure à 2,5 microns.

9. Fibre polymère fluorée selon l'une quelconque des revendications précédentes, **caractérisée en ce que** la seconde déformation de surface est une fente présentant une profondeur qui est supérieure à 10% d'une largeur moyenne de la fibre polymère fluorée ou supérieure à 25% d'une largeur moyenne de la fibre polymère fluorée.

10. Fibre polymère fluorée selon l'une quelconque des revendications précédentes, **caractérisée en ce qu'**elle comprend un corps allongé présentant une première extrémité et une seconde extrémité, et une fente s'étendant à travers la première extrémité du corps allongé.

11. Fibre polymère fluorée selon la revendication 10, **caractérisée en ce que** la fente comprend une première partie allongée qui est en partie enlevée d'une surface du corps allongé, la première partie allongée présentant une première extrémité couplée au corps allongé et une seconde extrémité libre et en option la fente comprend une seconde partie comportant une surface intérieure exposée du corps allongé et en option la surface intérieure exposée est plus rugueuse qu'une surface extérieure de la fibre polymère fluorée et comporte une multiplicité d'éléments incurvés de type fibrille s'étendant vers l'extérieur.

12. Fibre polymère fluorée selon la revendication 10 ou 11, **caractérisée en ce que** la fente s'étend à travers la seconde extrémité.

13. Fibre polymère fluorée selon la revendication 10, 11 ou 12, **caractérisée en ce que** la fente a une longueur qui est comprise entre 2% et 75% de la longueur de la fibre polymère fluorée, et la fente a de préférence une longueur qui est comprise entre 15% et 60% de la longueur de la fibre polymère fluorée.

14. Fibre polymère fluorée selon l'une quelconque des revendications précédentes, **caractérisée en ce que** la fente présente une profondeur qui est supérieure à 0,75 microns, de préférence supérieure à 2,0 microns.

15. Fibre polymère fluorée selon l'une quelconque des revendications précédentes, **caractérisée en ce que** la fibre polymère fluorée est une fibre de polytétrafluoroéthylène.

16. Fibre polymère fluorée selon l'une quelconque des revendications précédentes, **caractérisée en ce que** la fibre polymère fluorée est une fibre de flocage ou une fibre coupée.

17. Fibre polymère fluorée selon l'une quelconque des revendications 10 à 16, **caractérisée en ce que** la fibre présente une extrémité fendue, une surface intérieure exposée de la fibre polymère fluorée et une multiplicité d'éléments de type fibrille s'étendant vers l'extérieur à partir de la surface intérieure exposée.

18. Fibre polymère fluorée selon la revendication 17, **caractérisée en ce que** la fente a une profondeur d'au moins 0,8 microns.

19. Fibre polymère fluorée selon la revendication 17 ou 18, **caractérisée en ce que** la fente a une longueur qui est comprise entre 10% et 100% de la longueur de la fibre polymère fluorée et/ou l'extrémité de la fente apparaît effilochée.

20. Fibre polymère fluorée selon l'une quelconque des revendications 17 à 19, **caractérisée en ce que** la fibre de flocage polymère fluorée est une fibre polymère fluorée expansée ou une fibre de flocage de polytétrafluoroéthylène ou une fibre coupée de polytétrafluoroéthylène.

21. Procédé pour augmenter l'hydrophilicité de fibres polymères fluorées, **caractérisé en ce qu'**il comprend la modification mécanique des fibres polymères fluorées afin de créer une déformation de surface configurée de façon à procurer l'hydrophilicité améliorée, **en ce que** la déformation de surface est une fente présentant une profondeur qui est supérieure à 10% d'une largeur moyenne de la fibre polymère fluorée, et **en ce que** la fente est une déchirure qui s'étend en partie le long de la longueur de la fibre polymère fluorée, mais qui ne s'étend pas à travers une des extrémités opposées de la fibre.

22. Procédé selon la revendication 21, **caractérisé en ce que** la modification mécanique est effectuée en heurtant les fibres polymères fluorées entre elles et en option la modification mécanique est effectuée en entraînant les fibres polymères fluorées à l'intérieur d'un jet d'air et en option la modification mécanique est effectuée au moyen d'un broyeur à jets.

23. Procédé selon la revendication 21 ou 22, **caractérisé en ce que** la modification mécanique comprend la déchirure des fibres polymères fluorées et peut comprendre l'enlèvement partiel de parties de surface extérieures des fibres polymères fluorées et en option les parties de surface extérieures restent couplées par une de leurs extrémités aux fibres polymères fluorées d'où elles sont en partie enlevées.

24. Procédé selon la revendication 21 ou 22, **caractérisé en ce que** la modification mécanique comprend le refendage des fibres polymères fluorées en brins et/ou la réalisation d'une surface exposée rugueuse sur une partie des fibres polymères fluorées.

25. Procédé selon l'une quelconque des revendications 21 à 24, **caractérisé en ce que** la modification mécanique est effectuée en frappant les fibres polymères fluorées avec un jet d'air.

26. Procédé selon l'une quelconque des revendications 21 à 25, **caractérisé en ce que** les fibres polymères fluorées sont des fibres de flocage, des fibres coupées ou des combinaisons de celles-ci.

27. Procédé selon l'une quelconque des revendications 21 à 26, **caractérisé en ce que** la modification mécanique comprend la formation d'une fente dans une extrémité d'au moins une des fibres polymères fluorées, la fente présentant une longueur qui est comprise entre 5% et 100% de la longueur de ladite au moins une fibre polymère fluorée, ou en option la modification mécanique comprend la formation d'une fente dans une extrémité d'au moins une des fibres polymères fluorées, la fente présentant une longueur qui est comprise entre 10% et 90% de la longueur de ladite au moins une fibre polymère fluorée, ou en option la modification mécanique comprend la formation d'une fente dans une extrémité d'au moins une des fibres polymères fluorées, la fente présentant une longueur qui est comprise entre environ 20% et environ 50% de la longueur de ladite au moins une fibre polymère fluorée.

28. Procédé selon l'une quelconque des revendications 21 à 27, **caractérisé en ce que** la modification mécanique comprend la formation d'une déchirure dans au moins une des fibres polymères fluorées, la déchirure présentant une profondeur qui est supérieure à 1,0 micron, de préférence supérieure à 5,0 microns.

29. Procédé selon l'une quelconque des revendications 21 à 28, **caractérisé en ce que** la modification mécanique comprend la formation d'une multiplicité d'éléments de type fibrille qui s'étendent vers l'extérieur à partir d'une surface intérieure exposée d'au moins une des fibres polymères fluorées et/ou la modification mécanique ne raccourcit pas sensiblement une longueur totale d'une majorité des fibres polymères fluorées.

30. Procédé selon l'une quelconque des revendications 21 à 29, **caractérisé en ce que** le traitement comprend la formation d'au moins une déchirure à l'intérieur d'une surface de la fibre polymère fluorée, et ladite au moins une déchirure s'étend sensiblement en direction longitudinale le long de la surface de la fibre polymère fluorée et en option la formation de ladite au moins une déchirure comprend l'exposition d'une multiplicité de particules polymères fluorées sous-jacentes sensiblement alignées.

31. Procédé selon l'une quelconque des revendications 21 à 29, **caractérisé en ce que** le traitement comprend de refendage d'une extrémité de la fibre polymère fluorée en une multiplicité de brins et en option le traitement comprend le refendage d'une extrémité de la fibre polymère fluorée le long d'un grain de celle-ci en une multiplicité de brins.

32. Procédé selon l'une quelconque des revendications 21 à 31, **caractérisé en ce que** le traitement comprend la conversion d'une partie de surface lisse de la fibre polymère fluorée en une partie de surface rugueuse et en option la partie de surface rugueuse s'étend en direction longitudinale le long de la fibre polymère fluorée.

33. Procédé selon l'une quelconque des revendications 21 à 32, **caractérisé en ce qu'**on confère une hydrophilicité au matériau polymère fluoré en broyant mécaniquement le matériau polymère fluoré et en option le broyage mécanique comprend la projection d'un jet d'air dans le matériau polymère fluoré et en option le broyage mécanique comprend le passage du matériau polymère fluoré à travers un orifice d'un broyeur à jets avec au moins un jet d'air.

34. Procédé selon la revendication 33, **caractérisé en ce que** le broyage mécanique comprend le refendage d'au moins une extrémité d'une partie du matériau polymère fluoré en brins séparés, et/ou **en ce que** le broyage mécanique comprend la réalisation d'une surface rugueuse exposée sur une partie du matériau polymère fluoré et en option la surface rugueuse exposée s'étend le long d'un axe longitudinal du matériau polymère fluoré.

35. Procédé selon l'une quelconque des revendications 21 à 34, **caractérisé en ce que** le matériau polymère fluoré comprend des fibres de polytétrafluoroéthylène.
